

## UNITED STATES PATENT OFFICE.

GEORGE W. COLE, JR., OF PATERSON, NEW JERSEY.

## PROCESS OF TREATING SILK.

No Drawing. Application filed November 20, 1922. Serial No. 602,239.

*To all whom it may concern:*

Be it known that I, GEORGE W. COLE, Jr., a citizen of the United States, a resident of Paterson, in the county of Passaic and State 5 of New Jersey, have invented a certain new and useful Process of Treating Silk, of which the following is a specification.

This invention relates to a process of treating silk, and more particularly to a 10 process of treating silk before it is woven and dyed. The invention also includes the product of such a process.

The invention has as an object the weighting of silk before the socalled throwing or 15 twisting operation in order to incorporate the maximum quantity of the weighting material, such as a tin salt. The invention also has as an object the production of a well weighted silk that can be dyed in the piece 20 after the weaving operation. Another object of the invention is to weight silk with any suitable agent in such a manner as to incorporate the maximum amount of the weighting agent without interfering with 25 the other operations of the process. A still further object of the invention is to provide special means to facilitate the carrying out of the weighting and throwing operations. A still further object of the invention is to 30 arrange the other steps of the silk treating process so as to conveniently and effectively carry out the operations of weighting, throwing, weaving, and dyeing. Other objects of the invention will appear 35 from the following description.

My invention has made it possible for the first time to produce an undyed piece of woven silk goods in which is incorporated the maximum amount of weighting material, 40 and this has been accomplished by impregnating the silk in the skein before the socalled throwing operation. After the fabric has been completed by the weaving operation it need not be dyed at once but may 45 be kept in stock until the condition of the market determines what particular colors should be used in dyeing the goods. My product may be distinguished from other similar goods on the market by its very much 50 greater content of weighting material. In the preferred embodiment of the invention, the following procedure is adopted on the processing of 160 lbs. silk:

The silk as received in the skein in a raw 55 state and containing gum, is placed in a bath consisting of soft water, soap, sal soda,

and ammonia in the following proportions:—

600 gallons of water

30 lbs. green olive oil soap 60

5 lbs. sal soda

1 gallon ammonia

at 28° C. The purpose of this bath is to remove all foreign matters other than the natural gum from the silk. The time of immersion will vary from one to one and one-half hours. After the silk is removed from the bath, it is subjected to two washes of soft water of the same temperature as above and it is then subjected to another bath consisting of spring water and muriatic acid:—

600 gallons of water

3 gallons of muriatic acid.

This bath is given to the silk in order to remove whatever soap it may still contain and 75 it, furthermore, renders the silk receptive to the tin salt with which it is later brought in contact. After removal from the bath the silk is dried in an extractor and is then ready for the impregnating step.

The impregnation consists of a series of operations beginning with immersion in tin tetrachloride, and after one series of operations has been concluded the silk may again be subjected to repeated impregnations in order to bring the weight up to the desired percentage. However, only one series will be described, as follows: The silk is placed in a bath of tin tetrachloride, 28° Baumé glass, and allowed to remain there 80 for one hour, after which it is removed and extracted and washed with cold water on washing machines. It is then again extracted. It is next placed in a sodium phosphate bath, 600 gal. water, sodium phosphate 4 to 95 5° Baumé glass for about one hour and is then removed and washed twice with soft water, after which it is treated with spring water and muriatic acid, 600 gal. water and 3 gal. muriatic acid. After this washing, it 100 is again extracted.

The above tin weighting operation may, as aforesaid, be repeated from one to five times, according to the weight required, and after the conclusion of these treatments, the 105 silk is washed with water, extracted, and then given a sodium phosphate bath in which it remains for one hour. It is then washed three times with a solution of soft water and sal soda, 600 gal. water, 10 lbs. sal soda, 110 this treatment being followed with a sodium silicate bath, 600 gal. of water, sodium sili-

cate 4 to 5° Baumé glass, in which the silk remains for one hour, after which it is given three more soft water baths and then a bath of soda and ammonia—

5 600 gal. of water

40 lbs. sal soda

3 gal. ammonia

for one-half hour. This operation is then followed by another bath consisting of soft 10 water, green olive oil soap, and ammonia—

600 gal. of water

50 lbs. green olive oil soap

1 gal. ammonia

and the silk is allowed to remain in it for 15 one and one-half hours after which it is again washed with spring water and muriatic acid, extracted, and dried.

After these weighting operations and conditioning processes have been concluded, the 20 silk is forwarded to the throwster to be thrown, this latter operation consisting in giving the silk the particular number of twists per inch desired in the final woven product. This step is in itself known to 25 the art. Just before being subjected to this step in the process, the silk is treated with a solution made up by incorporating glycerine to the extent of five per cent (5%) in one hundred gallons of water and adding 30 thereto neat's-foot oil and soap to the extent of four per cent (4%) each for every hundred pounds of silk treated. The glycerine functions as a softening agent to facilitate the subsequent throwing operation 35 by keeping the silk fibers united and smooth, as otherwise they might tend to become disarranged, break off, or extend out from the individual threads to present a ruffled appearance.

40 After the so-called throwing operation the silk may be woven into a cloth and then dyed the various colors desired by manufacturers from time to time.

This dyeing operation need not be performed at once, as it may be carried out whenever a particular shade of color is desired by the public, and hence there will be no need for accumulating stores of silk dyed 45 goods having unmarketable colors. A dyeing operation is not performed, therefore, before the final step, as herein described, as there would not be any advantage in doing so. It could, however, be carried out at 50 an earlier stage if so desired.

55 The treatment with the glycerine solution constitutes a highly advantageous step of the process since it greatly facilitates the subsequent throwing operation and enables the manufacturer to produce a beautifully woven fabric. The weighting of the 60 silk before these operations is also of great advantage since it avoids disarrangement of the fibers in the skein and it is also possible to thereby incorporate more tin in each impregnation and in the final product, for

the immersion while in the skein renders it possible for the tin liquor to penetrate uniformly from all sides of the strands of silk.

A heavier weight can, therefore, be produced, which is of considerable advantage 70 and this can be produced before the throwing operation without in any way interfering with said throwing operation. It will therefore be apparent that by the combination of these steps in the manner described 75

I have improved considerably upon prior processes for treating silk and have made it possible to improve the qualities of the final product and to accomplish these results by improved process steps. 80

As many apparently widely different embodiments of this invention may be made without departing from the spirit thereof, it is to be understood that I do not intend to limit myself to the specific embodiment 85 thereof except as indicated in the appended claims.

It has been stated that an object of the invention is to weight the silk before the throwing operation, and the purpose of this 90 is to avoid any snarling or shriveling up which would occur if the weighting operation were attempted after the throwing operation. It is common in the art, however, to give raw silk a few turns before operating upon it in order to handle it better, this condition of the silk being termed "tram in the raw," and such a procedure may of course be adopted in the case of my process 95 also. Whether or not a preliminary twist 100 of a few turns is given will not change the subsequent order of steps which comprises the weighting operation while the silk is in the gum; and the subsequent throwing operation. 105

I claim:—

1. A process of treating silk comprising impregnating it with a tin solution, washing and drying it, treating it with a glycerine solution, throwing it, and weaving and dyeing it. 110

2. A process of treating silk comprising impregnating it with a metallic compound to weight it, treating it with a softening agent, throwing it, and dyeing it. 115

3. A process of treating silk comprising treating it in an aqueous alkaline bath containing soap, impregnating it in a tin solution, washing and drying it, treating it with a glycerine solution, throwing it to provide 120 a twist, and then weaving the silk.

4. A process of treating silk comprising treating it in an aqueous alkaline bath containing soap, impregnating it in a tin solution, treating it with a muriatic acid solution and washing it, treating it with a sodium silicate solution and washing it, drying it, soaking it in a glycerine solution, throwing it to provide a twist, and then weaving it. 125 130

5. A process of treating silk comprising impregnating it with a weighting material, treating it with a softening agent, throwing it, and weaving and dyeing the silk.
- 5 6. A process of treating silk comprising treating it in an aqueous alkaline bath containing soap, washing it with water, treating it with hydrochloric acid and drying it, soaking it in a solution of tin tetrachloride, 10 washing it, treating it with sodium phosphate solution and then washing it, treating it in a hydrochloric acid solution and then washing it, treating it with sodium phosphate solution and then washing it after the 15 conclusion of the weighting operation, treating it with an alkaline solution, followed by treatment with sodium silicate and washing, again treating it with an alkaline solution and then with an ammoniacal solution of a 20 green olive oil soap, washing it with a muriatic acid solution, drying it, soaking it in a glycerine and neat's-foot oil solution, throwing it to provide a twist, and weaving and dyeing the silk to form the finished 25 product.
7. A process of treating silk comprising treating it in an aqueous bath to remove foreign materials, drying it, impregnating it in a tin solution and thereafter washing it, 30 treating it with an alkaline solution and then drying it, soaking it in a glycerine solution to soften it, and then throwing and weaving the silk.
8. A process of treating silk comprising 35 impregnating it with a weighting material to give the desired weight to the silk while in the form of a skein before the weaving operation, throwing the silk to provide a twist of the desired number of turns per linear inch, and then weaving the silk.
9. A process of treating silk comprising 40 treating it in an aqueous bath to remove foreign materials, drying the silk, impregnating it with a weighting material to give the desired weight, washing and drying the silk, and then throwing and weaving it.
- 45 10. A process of treating silk comprising impregnating it with a weighting material to give it the desired weight, treating it with a softening agent to prevent the silk 50 from becoming rough during the throwing operation, and then throwing the silk to provide a twist.
11. A process of treating silk comprising impregnating it with a metallic compound 55 to weight it, treating it with a softening agent, throwing it, and dyeing it, these steps being performed in the order named.
12. A process of treating silk comprising impregnating it with a weighting material, 60 treating it with a softening agent, throwing it, and weaving and dyeing the silk, these steps being performed in the order named.
13. A process of treating silk comprising impregnating it with a weighting material 65 to give the desired weight to the silk while in the form of a skein before the weaving operation, throwing the silk to provide a twist of the desired number of turns per linear inch, weaving the silk, and then dye- 70 ing it.
14. A process of treating silk comprising treating it in an aqueous bath to remove foreign materials, drying the silk, impregnating it with a weighting material to give 75 the desired weight, washing and drying the silk, throwing and weaving it, and then dyeing it.
15. An undyed silk fabric comprising silk in the gum, and which contains over twenty- 80 five per cent of weighting material.
16. An undyed silk fabric comprising silk in the gum which contains over fifty per cent of weighting material.
17. A process of treating silk comprising 85 weighting it before degumming, weaving it, degumming and then dyeing it.
18. A process of treating silk comprising weighting it before degumming, throwing the silk, weaving it, degumming and then 90 dyeing it.

In testimony that I claim the foregoing, I have hereunto set my hand this 17th day of November, 1922.

GEORGE W. COLE, JR.